# EUROPEAN PATENT SPECIFICATION

(11) **EP 1 666 576 B1**
(45) Date of publication and mention of the grant of the patent: **23.07.2014**
(21) Application number: 04772782.1
(22) Date of filing: 03.09.2004
(51) Int. Cl.: C10M 171/02, C10M 173/02, B21B 25/04, C10M 103/00, C10M 103/06, C10M 145/40, C10N 10/02, C10N 20/02, C10N 30/00, C10N 30/06, C10N 40/24, C10N 50/02

(54) **LUBRICANT COMPOSITION FOR SEAMLESS STEEL PIPE WORKING**
SCHMIERMITTELZUSAMMENSETZUNG ZUR BEARBEITUNG VON NAHTLOSEN STAHLROHREN
COMPOSITION LUBRIFIANTE POUR L'USINAGE DE TUBES EN ACIER SANS SOUDURE

(30) Priority: 04.09.2003 JP 2003312232
(43) Date of publication of application: 07.06.2006
(73) Proprietor: Nippon Steel & Sumitomo Metal Corporation, Tokyo 100-8071 (JP)
(72) Inventor: Tanaka, Kazuo PALACE CHEMICAL CO., LTD., Yokohama-shi, Kanagawa 2360004 (JP); Mori, Shizuo PALACE CHEMICAL CO., LTD., Yokohama-shi, Kanagawa 2360004 (JP); Iida, Sumio SUMITOMO METAL INDUSTRIES, LTD., Osaka5410041 (JP)
(74) Representative: Simons, Amanda Louise
(86) International application number: PCT/JP2004/012833
(87) International publication number: WO 2005/023966

(56) References cited:
- EP-A- 0 839 895
- JP-A- 3 012 498
- JP-A- 2001 234 189
- JP-A- 2002 028 705
- DATABASE WPI Week 199722 Thomson Scientific, London, GB; AN 1997-241998 XP002523151 -& JP 09 078080 A (SUMITOMO METAL IND LTD) 25 March 1997 (1997-03-25)

## Description

### Technical Field

The present invention relates to a lubricant for hot rolling, which is mainly used for the production of a seamless steel pipe or tube by the Mannesmann process.

### Background Art

As is well known, in the production of a seamless metal pipe or tube by the Mannesmann process, a billet or bloom heated is made into a hollow blank with piercing mill, and then the hollow blank is finished into a product by means of a continuance mill (mandrel mill) and a sizing mill. On the step of elongation in Mannesmann process, inside face of a hollow blank is forcibly lubricated with a lubricant in order to prevent seizing. The lubricant is a graphite-based lubricant made mainly of granular graphite, scaly graphite, soil-form graphite or the like. It is used in a solid state or in the state of a liquid wherein a graphite is mixed with a binder.

In lubricity a graphite-based lubricant is suitable for hot rolling of a hard-to-work material such as stainless steel or high-alloy steel. However, the corrosion resistance of the material is hindered by carburization. Specifically, when a graphite-based lubricant is used for hot rolling of a hard-to-work material such as stainless steel or high-alloy, the inside face of a mother pipe or tube is carburized; therefore, grain boundaries due to grain-boundary - precipitation and the vicinity thereof are selectively corroded, so that the corrosion resistance thereof lowers, thereby losing the performance of product.

In order to improve this problem, Patent Document 1 suggests, instead of a conventional graphite-based lubricant, a lubricant composition based on a combination of an oxide-based layered compound, boric acid, and an alkali metal borate. Patent Document 2 suggests a lubricant composition' based on a combination of artificial mica, vermiculite or bentonite, Li, Na or K borate, a metaborate or pyroborate, and a hydrate thereof. These lubricants, wherein an oxide-based layered compound is combined with boric acid, are effective as non-carburizable lubricant that is excellent in lubricity.

On the other hand, non-carburizability is not required for ordinary graphite-based lubricant. Accordingly, these graphite-based lubricants can give the above-mentioned various properties when an ordinary organic thickener (for example, a water-soluble acrylic resin, or a water-soluble cellulose such as sodium carboxymethylcellulose) is sufficiently added to the graphite-based lubricants. For example, Patent Document 3 discloses a lubricant wherein both of a water-soluble polymer and a water-dispersible polymer are blended in large amounts, whereby the above-mentioned various properties are attained.
Patent Document 1: Japanese Patent Application Laid-Open (JP-A) No. 64-16894
Patent Document 2: JP-A No. 5-171165
Patent Document 3: JP-A No. 2-51592

EP-A-0 839 895 discusses a lubricant for use in hot work tools such as cross-roll rolling of a seamless steel pipe. JP-A-978080 describes a lubricant composition for high temperature working which is obtained by blending one or more particular oxide-based layer materials selected from potassium tetrasilicic mica, sodium tetrasilicic mica, natural phlogopite, bentonite, montomorillonite and vermiculite with one or more binders selected from boron oxide, boric acid, an alkali metal borate, sodium carbonate, potassium carbonate and sodium silicate or potassium silicate.

### Disclosure of the Invention

### Problems to be Solved by the Invention

The lubricants disclosed in the Patent Documents 1 and 2 are supplied in a solid state onto a face of a tool (for example mandrel bar), or are applied to a tool in a state that they are dispersed into water. Accordingly, in order to use the lubricants in a continuance mill (mandrel mill), it becomes necessary that they have various properties totally, such as storage stability before use, transferability inside an apparatus tube, sprayability to a lubricated site, and property of uniform adhesion to a high - temperature mandrel bar. However, it is difficult Lo attain these properties totally.

In elongating a hollow blank of stainless steel or high-alloy steel by a continuance mill(mandrel mill), non-carburizability is persistently required in order to keep corrosion resistance thereof. Thus, the above-mentioned polymers cannot be blended in large amounts.

Accordingly, an object of the present invention is to provide a lubricant composition which totally has various properties, such as storage stability, transferability inside an apparatus tube, sprayability to a lubricated site, and property of uniform adhesion to a high-temperature mandrel bar without losing non-carburizability or excellent lubricity in elongating hard-to-work materials (for example, such as 13 chromium steel and stainless steel) by a continuance mill(mandrel mill).

### Means for Solving the Problems

The present invention is a lubricant composition for seamless steel pipes or tubes working which has a viscosity property represented by the following approximate expression: $Y = a ⋅ {X}^{b}$
wherein Y: viscosity (mPa·s), X: shear rate (s⁻¹) ; and
a: 4000 to 40000 and b: -1.0 to -3.0 while a lubricant composition is stored still, and a: 1000 to 20000, and b: -1.0 to -0.15 after 90 seconds from the time when shearing a lubricant composition is finished.

The wording "90 seconds from the time when shearing a lubricant composition is finished" means the time of 60 seconds after the following measurement start: a lubricant composition is stirred; and at 30 seconds from the end of the stirring, the viscosity of lubricant composition is measured at a given shear rate. Consequently, the wording "90 seconds" corresponds to the total value of the above-mentioned 30 seconds and 60 seconds. The wording "the time when shearing a lubricant composition is finished" means the time when the above-mentioned stirring operation is finished.

The lubricant composition for seamless steel pipes or tubes working comprises 10 to 40% by mass of an oxide-based layered compound, 5 to 30% by mass of one or more alkali metal salts or amine salts of boric acid, 0.11 to 3.0% by mass of one or more water-soluble polymers which are soluble in an aqueous solution of the alkali metal salt (s) or amine salt (s) of boric acid, and water as the balance.

It is preferred that the lubricant composition for seamless steel pipes or tubes working comprises, as water-soluble polymer(s), a pseudo plastic fluidity water-soluble polymer, or a pseudo plastic fluidity water-soluble polymer and a thixotropic fluidity water-soluble polymer.

Alternatively, it is preferred that the lubricant composition for seamless steel pipes or tubes working comprises, as water-soluble polymer(s), a pseudo plastic fluidity water-soluble polymer in an amount of 0.01 to 1.0% by mass of the whole of the lubricant composition, and a thixotropic fluidity water-soluble polymer in an amount of 0.1 to 2.0% by mass of the whole of the lubricant composition.

### Effects of the Invention

According to the invention, it is possible to provide a lubricant composition for seamless steel pipes or tubes working which totally has various properties, such as storage stability, transferability inside an apparatus tube, sprayability to lubricated sites, and property of uniform adhesion to a high-temperature mandrel bar without losing non-carburizability or excellent lubricity to hard-to-work materials such as 13 chromium steel and stainless steel.

### Best Mode for Carrying Out the Invention

An oxide-based layered compound used as main agent in a lubricant composition for seamless steel pipes or tubes working of the invention is, for example, any natural mica or artificial mica. Examples of the mica include:
Potassium tetrasilicone mica {KMg_{2.5}(Si₄O₁₀)F₂},
Sodium tetrasilicone mica {NaMg_{2.5}(Si₄O₁₀)F₂}, and
Natural golden mica {KMg₃(AlSi₂O₁₀)(OH)₂}.
In the lubricant composition for seamless steel pipes or tubes working of the invention, one or more therefrom can be used. Instead of the mica, or together with the mica, vermiculite, bentonite or the like can be used. Sodium tetrasilicone mica is the most preferable for the lubricant composition for seamless steel pipes or tubes working of the invention.

The average particle diameter of the oxide-based layered compound is from 1 to 40 µm, preferably from 5 to 30 µm. If the particle diameter is too small, the effect of interlayer slip becomes small. On the other hand, if the particle diameter is too large, problems such that a nozzle is blocked when the lubricant composition is sprayed are caused. The adding amount of the oxide-based layered compound is from 10 to 40% by mass of the lubricant composition of the lubricant of the invention for seamless steel pipes or tubes working, preferably from 20 to 30% by mass thereof. If the adding amount of the oxide-based layered compound is too small, the seizing resistance becomes low so that a problem is caused about the lubricity thereof. On the other hand, if the adding amount of the oxide-based layered compound is too large, the viscosity of the lubricant composition becomes too high so that a problem is caused about the workability.

Alkali metal salt(s) or amine salt(s) of boric acid in a lubricant composition help (s) the oxide-based layered compound, which is a main agent, spreading on a high-temperature mandrel bar, or the salt(s) itself/themselves work(s) as a single or plural lubricating auxiliaries. Examples of the alkali metal salt(s) of boric acid include lithium borate, sodium borate, andpotassiumborate. Ametaborate, a pyroborate and/or a hydrate, such as borax (Na₂Ba₄O₇·10H₂O) can be used.

The adding amount of alkali metal salt (s) or amine salt (s) of boric acid into the lubricant composition is from 5 to 30% by mass, preferably from 10 to 20% by mass. If the adding amount of the salt (s) is too large, the salt (s) hinder (s) the lubricity of the main agent. If the adding amount of the salt(s) is too small, it hinders a main object, that is, the property of uniform adhesion to a mandrel bar caused by the main agent. Moreover, the lubricity is insufficient, so that shortage of lubricity is induced.

Aswater-solublepolymer(s) usedinalubricantcomposition for seamless steel pipes or tubes working of the invention, the following can be used: a single or a combination of two or more selected from natural, semi-natural and synthetic water-soluble polymers having the viscosity conditions prescribed in the present invention. These water-soluble polymers will be specifically described later.

Next, an ideal viscosity which has been found by the present inventors is shown in FIG. 1. FIG. 1, wherein viscosity is represented by its vertical axis and time is represented by its horizontal axis, is a graph of the viscosity variation of a lubricant composition changed with time under the following conditions:
(i): a lubricant composition is kept still,
(ii) to (iii): a lubricant composition is sheared at a constant rate, and
(iii) to (iv) : the shearing of a lubricant composition is finished.

The inventors have found out that a lubricant composition of which viscosity property is as the following (1) to (4), has excellent lubricity in the production of a seamless metal pipe or tube according to the Mannesmann process:
(1) In order to store a lubricant in a state that solid particles of the oxide-based layered compound is even and stable, the viscosity at the time (i) when a lubricant composition is kept still has to be high. If the viscosity is low, the solid particles settle down.
(2) In order to keep the transferability inside an apparatus tube and the sprayability, the viscosity at the time (ii) to (iii) when a lubricant composition is sheared needs to be low.
(3) For the property of fine and even adhesion to a high-temperature bar, which gives a great influence on lubricity, the viscosity at the time (ii) has to be high. From a microscopic viewpoint, a lubricant is continuously sprayed and adheres onto a tool surface. On a coat of lubricant adhered formerly, a lubricant sprayed later arrives. That is, a coat of lubricant adhered formerly is sheared. Accordingly, if the viscosity at the time (ii) is low, the lubricant is unfavorably peeled down or scattered by the pressure of spraying lubricant.
(4) In order to keep uniform and stable retention property of the solid particles on a tool surface, the viscosity needs to rise immediately after the finish of the shearing at the times of (iii) to (iv). If it takes much time that the viscosity recovers or the viscosity does not recover, the lubricant unfavorably flows down from the tool surface.

In order to realize that a lubricant has the viscosity showed as FIG, 1, and attains various properties, such as storage stability, transferability inside an apparatus tube, sprayability to lubricated sites, and property of uniform adhesion to a high-temperature mandrel bar without adding a large amount of a polymer, the inventors have found out that the lubricant viscosity has to fulfill the expression describedbelow. In other words, the inventors have measured the viscosity property of the present invention lubricant having the above-mentioned various properties by a viscosity-measuring method described in Examples which is described later, so as to find that the parameters a and b which are counted from the measured viscosity curve has to be within the range described in the following approximate expression: $Y = a ⋅ {X}^{b}$
wherein Y: viscosity (mPa·s), X: shear rate (s⁻¹); and
a: 4000 to 40000 and b: -1.0 to -0.3 while a lubricant composition is stored still; and
a: 1000 to 20000, and b: -1.0 to -0.7.5 after 90 seconds from the time when shearing a lubricant composition is finished.

In the approximate expression: $Y = a ⋅ {X}^{b} ,$
a and b are set into the range of 4000 to 40000 and that of -1.0 to -0.3, respectively, while a lubricant composition is stored to be kept still. If a is less than 4000, the viscosity of a lubricant composition is low while a lubricant composition is kept still. Consequently, the oxide-based layered compound settles down while a lubricant composition is stored. If a is more than 40000, the fluidity of a lubricant composition is substantially lost, so as to cause a problem about the transfer thereof.

Further, if b is more than -0.3, the difference between the viscosity of a lubricant composition while it is kept still and that while a lubricant composition is sheared (i.e., transferred or sprayed) is small, so as to cause a problem about the transfer or spray thereof. If b is less than -1.0, the viscosity of a lubricant composition becomes too low when it is sprayed. Consequently, at the time of applying a lubricant composition onto a tool, the lubricant adhered formerly is peeled down or scattered by the pressure of spraying lubricant itself. More preferably a and b are as follows:
a: 7000 to 30000, and
b: -0.5 to -0.8.

The approximate expression: Y = a·X^{b} is described herein with reference to FIG. 1. As the value a is larger and the value b is smaller while a lubricant composition is stored still (that is, when the value X is limitlessly near 0), the viscosity at the time (i) in FIG. 1 is higher so that the stability is better. For example, in the case of X = 0.01, a = 100000 and b = -1, Y = 10,000,000 mPa·s.

In the approximate expression: $Y = a ⋅ {X}^{b} ,$
a and b are set into the range of 1000 to 20000 and that of -1.0 to -0.15, respectively,
after 90 seconds from the time when shearing a lubricant composition is finished. If a is less than 1000 or b is less than -1.0, the water-soluble polymer (s) is /are sheared and thus it takes much time that the viscosity recovers. Alternatively, a lubricant composition is sheared and its viscosity does not recover, and at this time the lubricant flows down. If a is more than 20000 or b is more than -0.15, a problem is caused when a lubricant composition is transferred or sprayed. More preferably, a and b are as follows:
   a: 3000 to 20000, and
   b: -0.3 to -0.8.

As the value a is larger and the value b is smaller while a lubricant composition is sheared (that is, when the value X is larger immediately after a lubricant composition is stirred), the viscosity at the time (ii) and (iii) in FIG. 1 is higher. If a is too large and b is too small, the viscosity does not become low and that hinders the transferability and sprayability. For example, in the case of X = 10, a = 100000 and b = -1, Y = 10,000 mPa·s.

The time after a lubricant composition is sheared (that is, when the value X just after the stirring is small) is (iv) in FIG. 1. In the case that numerical values of a and bare similar to the numerical values when a lubricant composition is stored still, the viscosity rapidly recovers. In this case, the lubricant that adheres to a tool does not easily flow down. Accordingly, such an appropriate viscosity property as in the invention described above is crucial.

The inventors have made eager investigations on conditions for attaining the above-mentioned viscosity property, so as to find out the following: the use of only a pseudo plastic fluidity water-soluble polymer, as the water-soluble polymer(s) used in a lubricant composition of the invention, may cause the above mentioned property to be attained; however, the addition of both of a pseudo plastic fluidity water-soluble polymer and a thixotropic fluidity water-soluble polymer easily causes the above mentioned property to be attained.

Typical examples of the pseudo plastic fluidity water-soluble polymer include bio-gums such as xanthan gum, welan gum and ramsan gum. The chemical structure of xanthan gum is a water-soluble polymer polysaccharide wherein linking blocks each having two glucoses, two mannoses and one glucuronic acid as constituents are recurred. A model of the chemical structure is illustrated in FIG. 2.

Typical examples of the thixotropic fluidity water-soluble polymer include carboxymethylcelulose salts (Na, K, and amine salts). As an example thereof, a chemical structure model of a long-chain polymer wherein glucoses are subjected to glucoside bonding is illustrated in FIG. 3.

Pseudo plastic fluidity and/or thixotropic fluidity can also be attained by incorporating, into a lubricant composition, one or more selected from the following materials which are different from the above and cannot be easily distinguished from each other dependently on the molecular weight, another component or other components (for example, a metal (such as Ca) ion), or pH: bio-gums such as gellan gum, and succinoglucan; natural polysaccharides such as tamarind, tara gum, locust bean gum, and carrageenan; cellulose derivatives such as methylcellulose, ethylcellulose, hydroxyethylcellulose, hydroxypropylcellulose, hydroxyethylmethylcellulose, and hydroxypropylmethylcellulose; polyacrylic acid salts (Na, K, and amine salts), and alginic acid salts (Na, K, and amine salts).

Next, the viscosity property of a pseudo plastic fluidity water-soluble polymer in static and dynamic states is shown in FIG. 4, and that of a thixotropic fluidity water-soluble polymer is shown in FIG. 5. According to only the pseudo plastic fluidity water-soluble polymer, a change from the static state to the dynamic state is like a straight line. Thus, the change comes under the scope of the invention, but satisfaction is not sufficiently given. On the other hand, the viscosity change of the thixotropic fluidity water-soluble polymer, wherein the viscosity difference from the static state to the dynamic state is small, is gentler than the viscosity change of the pseudo plastic fluidity water-soluble polymer. About the thixotropic fluidity water-soluble polymer, some amount of time (yield value) is necessary from the start of the dynamic state to a drop in the viscosity. About the thixotropic fluidity water-soluble polymer, time is also necessary for a rise in the viscosity in the case that the dynamic state is shifted to the static state. In the case that time is required for such a viscosity change, the lubricant sprayed onto a mandrel bar cannot undergo viscosity change for ideal film-formation in a film-forming step from the spray to drying. As a result, the lubricant does not adhere evenly onto the mandrel bar at ease. Accordingly, the object of the invention cannot be sufficiently realized by only the thixotropic fluidity water-soluble polymer.

In order to realize the ideal viscosity form shown in FIG. 1, it is desired to add the above-mentioned two polymers together. Specifically, the addition percentage of the pseudo plastic fluidity water-soluble polymer is from 0.01 to 1.0% by mass of the whole of the lubricant composition and the addition percentage of the thixotropic fluidity water-soluble polymer is from 0.1 to 2.0% by mass of the whole of the lubricant composition. More preferably, the addition percentage of the pseudo plastic fluidity water-soluble polymer is from 0.05 to 0.5% by mass of the whole of the lubricant composition and in connection therewith the addition percentage of the thixotropic fluidity water-soluble polymer is from 0.5 to 1.5% by mass of the whole of the lubricant composition. If the addition percentage of the pseudo plastic fluidity water-soluble polymer gets larger than that of the thixotropic fluidity water-soluble polymer, the viscosity change by shear becomes too large so that a lubricant composition does not adhere evenly onto a mandrel bar at ease. If the percentage of the thixotropic fluidity water-soluble polymer becomes too large, the dispersion stability of the oxide-based layered compound and the spreading property to a high-temperature mandrel bar are deteriorated so that the property of the uniform adhesion gets worse.

A lubricant which includes each fluidity water-soluble polymer of the above-mentioned two has a mixed viscosity property of that shown in FIG. 4 and FIG. 5. A qualitative viscosity property thereof is as follows: in FIG. 1, at time(i)when a lubricant composition is kept still, the viscosity is high because of the nature of the pseudo plastic fluidity water-soluble polymer; when shear is applied thereto thereafter, a drop in the viscosity at (i) to (iii), having a synthetic form of pseudo plastic fluidity and thixotropic fluidity states, is exhibited; and at last the viscosity property is converted into a rise in the viscosity shown at (iv) immediately after shearing is finished.

If the total percentage of the two polymers is more than 3.0% by mass of the total of a lubricant composition, a problem of carburization is unfavorably caused. If the percentage of the two polymers is less than 0.11% by mass of the total of a lubricant composition, the dispersion stability of the oxide-based layered compound is deteriorated so that the resultant is not suitable for a lubricant composition of the invention.

The addition of an ordinary antifoaming agent or dispersing agent causes a risk of carburization if the agent is an organic compound; therefore, the addition of a small amount (0.5% or less by mass of the total of the lubricant composition) thereof is permissible. Inorganic agents, which do not contain carbon, are allowed to be added as long as the agents do not give a significant influence onto basic performances of the invention.

### Examples

### (1) Preparations of samples for evaluation

Eighteen working examples shown in Tables 1 to 2 and 10 comparative examples shown in Table 3, that is, 28 samples in total were prepared. Tables 1 to 3 also show peculiar numeric constants "a" and "b" in the approximate expressions of these samples while they were stored still, and those after 90 seconds from the time when shearing thereto was finished.

### (2) Performance-evaluating tests

### 1) Viscosity

### (i) Measuring conditions

Measuring device: Model-B viscometer (Toki Sangyo Co., Ltd) was used.
Measuring temperature: It was set to 25°C.
Shearing conditions:
a 500-mL of the samples were respectively put into a 500-mL beaker, and then stirred at 3000 rpm for 1 minute by means of a propeller of 50 mm diameter.
Rotation number:
   Low rotation (1.5 rpm) [shear rate: 0.323 to 0.366 S⁻¹]
High rotation (60 rpm) [shear rate: 12.9 to 14.6 s⁻¹]

### (ii) Measuring method

Stationary viscosity: After each of the samples was stirred and kept still for 24 hours, it started to measure the viscosity at low shear rate. After 60 seconds from the start of the measurement, data of the viscometer was read out and was multiplied by a coefficient. Subsequently, it started to measure the viscosity at high shear rate. After 60 seconds from the start of the measurement, data of the viscometer was read out and was multiplied by a coefficient. The result was recorded as stationary viscosity.

Shear viscosity: Each of samples was stirred to shear thereto with the propeller. After 30 seconds from the finish of shearing, it started to measure the viscosity at low shear rate. After 60 seconds from the start of the measurement, data of the viscometer was read out and was multiplied by a coefficient. The sample was again stirred, and after 30 seconds therefrom it started to measure the viscosity at high shear rate. After 60 seconds from the start of the measurement, data of the viscometer was read and was multiplied by a coefficient. The result was recorded as shear viscosity.

In the measurements, the time "90 seconds from the time when shearing was finished (or after 90 seconds from the finish of the shearing)" means the time of 60 seconds after the following measurement start: an operation of shearing a sample was performed by stirring the lubricant composition; and after 30 seconds from the finish of the operation, it started to measure the viscosity at a given shear rate. Thus, the time "90 seconds" corresponds to the total value of the above-mentioned 30 seconds and 60 seconds. The "time when shearing was finished (or the time of the finish of the shearing" means the time when rotating the propeller for the above-mentioned stirring is stopped.

### (iii) Decision of the peculiar numeric constants "a" and "b"

Logarithms of both sides of the approximate expression Y = a·X^{b} are given as follows: log(Y) = blog(X) + log (a)

According to X and Y obtained in the above-mentioned measurements, log (X) and log (Y) are calculated. These are plotted in a graph corresponding to its vertical axis and its horizontal axis, respectively. As a result, there is a substantially linear relationship (relationship of a linear function) between them. From the graph, "b", which is the gradient of the linear function and "a", which is the vertical axis intercept, can be obtained by the least-squares method.

### 2) Storage stability

### (i) Test method

The samples were respectively stored in a 500-mL glass container, and kept still for 7 days. Thereafter, a state of separation thereof was observed.

(ii) Evaluating method: The samples were evaluated in accordance with the following evaluating criterion:
⊚: No supernatant was generated, and no sedimentation was caused on the bottom.
○: Supernatant was generated in an amount of less than 5%, and no sedimentation was caused on the bottom.
Δ: Supernatant was generated in an amount of 5% or more, and no sedimentation was caused on the bottom.
x: Sedimentation was caused on the bottom regardless of the generation of supernatant.

The word "supernatant" means a substantially transparent liquid portion containing no solid. By observing a beaker of sample from a side-direction, the height of a supernatant in the beaker is measured. The height of a supernatant in the beaker was evaluated as the percentage thereof into the height of the liquid in the beaker.

The wording "sedimentation on the bottom" means a state that a solid lubricant settles down on the bottom and thus a hard layer having no fluidity can be perceived.

### 3) Carburization

### (i) Test method

Four examples 4, 11 and 13 and Comparative Examples 6 were respectively sprayed and applied onto a mandrel bar made of SKD61 and having an outer diameter of 140.5 mm and an effective portion length of 18 m, and then dried and solidified to form a substantially uniform lubricant coat having a film thickness of 100 µm on the surface of the mandrel bar. The mandrel bar, onto which the lubricant was applied, was inserted into an hollow shell. Continuance mill (mandrel mill) composed of 7 stands was used to roll a hollow blank into an mother pipe or tube.

Specification of a hollow blank before elongation:
Material: Austenite stainless steel (SUS304L);
Working: piercing by piercing mill with inclined-roll;
Shape: outer diameter: 181.0 mm, thickness: 16.0 mm, and
length: 7000 mm.
Shape of a mother pipe or tube after elongation:
Outer diameter: 151.0 mm, thickness: 5.0 mm, and
length: 25300 mm.

After the hollow blanks were respectively rolled with continuance mill (mandrel mill), the mother pipe or tube was rolled to determined outer diameter by sizing mill. A product had an outer diameter of 63.5 mm, thickness of 7.0 mm and a length of 40000 mm. An arc-form test piece having a thickness of 5 mm, a width of 25 mm and a length of 50 mm was made from a product. This test piece was used to make a sulfuric acid-copper sulfate corrosion test prescribed in JIS G0575, and then the state of a grain boundary corrosive crack generated in the inside surface was observed.

(ii) Evaluating method: An evaluation was made in accordance with the following criterion:
⊚: No crack.
x: A crack was generated.

### 4) Sprayability

### (i) Test conditions

Spray manner: an airless spray.
Spraying pressure: It was set to 3.0 MPa.
Nozzle: 1/4MVVP5010 (manufactured by Kabushiki Kaisha Ikeuchi (transliteration)).
Spray pattern: Fan-shaped
Spray angle:
50 degrees (angle at which water was spread into a fan shape when water was sprayed)
Sample temperature: It was set to 25°Ctomake an evaluation.

(ii) Evaluation: The spreading property was evaluated by measuring the spray angle. The result of the evaluation was recorded in accordance with the following evaluating criterion:
⊚: The spray angle was a almost predetermined angle (50 degrees).
O: The spray angle was somewhat narrower than the predetermined angle (40 to 45 degrees).
Δ: The spray angle was far narrower than the predetermined angle (20 to 39 degrees).
x: The spray angle was hardly spread (less than 20 degrees), or sprayed particles were large.

### 5) Adhesion property (adhesion amount)

### i) Test conditions

Spray manner: an airless spray.
Spraying pressure: It was set to 3.0 MPa.
Nozzle: 1/4MVVP5010 (manufactured by Kabushiki Kaisha Ikeuchi (transliteration)).
Spray angle: 50 degrees
Test piece temperatures: The temperatures were set to 60, 80, 100, and 120°C.
Nozzle/test-piece distance: It was set to 250 mm to make the test.
Test speed: It was set to 2 m/second.

(ii) Evaluating method: Each sample was sprayed onto a test piece (a 65 mm x 120 mm x 30 mm steel plate) under the test conditions. After spraying, the test piece was heated up to 120°C to dry the lubricant . Thereafter, the test piece naturally cooled down to 20-40°C. The lubricant coat was shaved off with a knife and its weight was measured. The weight of the coat was divided by the adhesion area (0.0078 m²) and the result was defined as the adhesion amount. It was evaluated in accordance with the following evaluating criterion:
⊚: The coat adhered evenly, and the adhesion amount was 50 g/m² or more.
○: The coat adhered substantially evenly, and the adhesion amount was 50 g/m² or more.
Δ: The lubricant somewhat flowed down, and the adhesion amount was 40 g/m² or more.
x: The lubricant flowed down largely, and the adhesion amount was 30 g/m² or less.
xx: The adhesion property was bad because of repellency, and the adhesion amount was 30 g/m² or less.

### (3) Test results

The results of the tests 1) to 5) are shown in Tables 1 to 3.

**[Table 1]**

| | | Example 1 | Example 2 | Example 3 | Example 4 | Example 5 | Example 6 | Example 7 | Example 8 | Example 9 |
|---|---|---|---|---|---|---|---|---|---|---|
| Sodium tetrasilicone mica | | 10.00 | 10.00 | 20.00 | 15.00 | 20.00 | 20.00 | 20.00 | 20.00 | 30.00 |
| Natural golden mica | | | | | | | | | | |
| Bentonite | | | | | | | | | | |
| Potassium borate | | | 10.00 | 13.00 | 8.00 | 10.00 | 10.00 | 15.00 | 15.00 | 12.00 |
| Amine borate | | 5.00 | 5.00 | | 8.00 | | 5.00 | 500 | 5.00 | 3.00 |
| Xanthan gum | | 050 | 040 | 0.70 | 0.10 | | 0.40 | 0.50 | 0.30 | 0.30 |
| Welan gum | | | | | | 0.05 | | | | |
| CMC (A) | | 050 | | | | | | 0.50 | | |
| CMC (B) | | | 050 | | | | | | | 0.30 |
| CMC (C) | | | | | 1.00 | 1.00 | | | 050 | |
| CMC (D) | | | | | | | | | | |
| Na polyacrylate (A) | | | | | | | | | | |
| Na polyacrylate (B) | | | | | | | 020 | | | |
| Water (Calculated amount) | | 84.00 | 74 10 | 66.30 | 67.90 | 68.95 | 6440 | 59.00 | 59.20 | 54 40 |
| Liquid state | | | | | | | | | | |
| Stationary viscosity | (low shear rate) | 18850 | 15930 | 53500 | 14180 | 15400 | 15800 | 22080 | 26000 | 30900 |
| | (high shear rate) | 1080 | 1390 | 1750 | 1780 | 1870 | 1040 | 1720 | 1700 | 1860 |
| After shearing | (low shear rate) | 19520 | 17400 | 48420 | 6325 | 2250 | 18900 | 25000 | 18000 | 24130 |
| | (high shear rate) | 1090 | 1410 | 1690 | 1410 | 1170 | 1060 | 1630 | 1600 | 1710 |
| | | | | | | | | | | |
| At a time of stationary storage | (coefficient a) | 8154 | 7795 | 19638 | 7719 | 8302 | 7119 | 10451 | 11691 | 13562 |
| | (coefficient b) | -0.777 | -0.663 | -0.929 | -0.564 | -0 573 | -0.739 | 0.693 | 0741 | -0.763 |
| Immediately after the shearing | (coefficient a) | 8380 | 8332 | 18115 | 4074 | 1858 | 8125 | 11232 | 8856 | 11110 |
| | (coefficient b) | -0.784 | -0.683 | -0.911 | -0.408 | -0.178 | -0 783 | -0.742 | 0.657 | -0.719 |
| | | | | | | | | | | |
| Storage stability | | ⊚ | ⊚ | ⊚ | ⊚ | ⊚ | ⊚ | ⊚ | ⊚ | ⊚ |
| Carburization | | ⊚ | ⊚ | ⊚ | ⊚ | ⊚ | ⊚ | ⊚ | ⊚ | ⊚ |
| Sprayability | (25°C) | ⊚ | ⊚ | ○ | ⊚ | ⊚ | ○ | ⊚ | ⊚ | ⊚ |
| Adhesive property | (60°C) | ⊚ | ⊚ | ⊚ | ○ | ○ | Δ | ⊚ | ⊚ | ⊚ |
| | (80°C) | ⊚ | ⊚ | ⊚ | ⊚ | ○ | Δ | ⊚ | ⊚ | ⊚ |
| | (100°C) | ⊚ | ⊚ | ⊚ | ⊚ | ⊚ | ○ | ⊚ | ⊚ | ⊚ |
| | (120°C) | ⊚ | ⊚ | ○ | ⊚ | ⊚ | ○ | ⊚ | ⊚ | ⊚ |

**[Table 2]**

| | | Example 10 | Example 11 | Example 12 | Example 13 | Example 14 | Example 15 | Example 16 | Example 17 | Example 18 |
|---|---|---|---|---|---|---|---|---|---|---|
| Sodium tetrasilicone mica | | 40.00 | | | 10.00 | | 5.00 | 5.00 | | 20.00 |
| Natural golden mica | | | 2000 | | 10.00 | 10.00 | 5.00 | 5.00 | 10.00 | |
| Bentonite | | | | 20.00 | | 1000 | 5.00 | 5.00 | | |
| Potassiim borate | | 12.00 | 12.00 | 1000 | 10.00 | 2000 | 5.00 | 5.00 | 30.00 | 30.00 |
| Amine borate | | 3.00 | 300 | 10.00 | 5.00 | | 10.00 | 1000 | | |
| Xanthan gum | | | 0.60 | | | | | 0.10 | 020 | |
| Welan gum | | 005 | | 0.15 | 020 | 0.15 | 0.10 | | | 0.02 |
| CMC (A) | | | | | 1.50 | | | | | |
| CMC (B) | | | | | | | | | | 0.50 |
| CMC (C) | | | | | | | 1.00 | 1.00 | 1.00 | |
| CMC (D) | | 050 | | | | | | | | |
| Na polyacrylate (A) | | | 2.00 | | | 1.00 | | | | |
| Na polyacrylate (B) | | | | 0.30 | | | | | | |
| Water (Calculated amount) | | 44.45 | 62.40 | 59.55 | 63.30 | 58.85 | 68.90 | 68.90 | 58.80 | 49.48 |
| Liquid state | | | | | | | | | | |
| Stationary viscosity | (low shear rate) | 12070 | 42400 | 32000 | 45100 | 17800 | 50000 | 9500 | 18000 | 9225 |
| | (high shear rate) | 1740 | 2480 | 1450 | 4230 | 1650 | 3050 | 1800 | 2150 | 1680 |
| After shearing | (low shear rate) | 8920 | 32100 | 17500 | 9830 | 7200 | 8500 | 5800 | 133300 | 1975 |
| | (high shear rate) | 1580 | 2500 | 1100 | 2230 | 900 | 2100 | 1560 | 1980 | 835 |
| | | | | | | | | | | |
| At a time of stationary storage | (coefficient a) | 6843 | 18453 | 12923 | 22542 | 8866 | 22031 | 5835 | 9657 | 5600 |
| | (coefficient b) | -0.526 | 0771 | -0.841 | -0.643 | 0.646 | -0.76 | -0.452 | -0.577 | -0.463 |
| Immediately after the shearing | (coefficient a) | 5371 | 15193 | 7779 | 6364 | 3915 | 5643 | 3947 | 7611 | 1534 |
| | (coefficient b) | -0.47 | -0.693 | -0.752 | 0.403 | -0.565 | -0.38 | -0.357 | -0.517 | 0.234 |
| | | | | | | | | | | |
| Storage stability | | ⊚ | ⊚ | ⊚ | ⊚ | ○ | ⊚ | ⊚ | ⊚ | ○ |
| Carburization | | ⊚ | ⊚ | ⊚ | ⊚ | ⊚ | ⊚ | ⊚ | ⊚ | ⊚ |
| Sprayability | (25°C) | ⊚ | ⊚ | ○ | ○ | ⊚ | ⊚ | ⊚ | ⊚ | ⊚ |
| Adhesive property | (60°C) | ⊚ | ⊚ | Δ | ⊚ | ○ | ⊚ | ⊚ | ⊚ | Δ |
| | (80°C) | ⊚ | ⊚ | Δ | ⊚ | ○ | ⊚ | ⊚ | ⊚ | Δ |
| | (100°C) | ⊚ | ○ | ○ | ⊚ | ⊚ | ⊚ | ⊚ | ⊚ | ○ |
| | (120°C) | ⊚ | Δ | ○ | ⊚ | ○ | ⊚ | ⊚ | ⊚ | Δ |

**[Table 3]**

| | | Comparative Example 1 | Comparative Examples 2 | comparative Example 3 | Comparative Example 4 | Camparative Example 5 | Comparative Example 6 | Comparative Example 7 | Comparative Example 8 | Comparative Example 9 | Comparative Example 10 |
|---|---|---|---|---|---|---|---|---|---|---|---|
| Sodium tetrasilicone mica | | 20.00 | 30.00 | | | 20.00 | 10.00 | 20.00 | 7.00 | 42.00 | |
| Natural golden mica | | | | 15.00 | 50.00 | | 10.00 | | | | 20.00 |
| Bentonite | | | | | | 10.00 | | | | | 10.00 |
| Potassium borate | | 10.00 | | 5.00 | 30.00 | 10.00 | 15.00 | 2000 | 200 | 3000 | 10.00 |
| Amine borate | | | 10.00 | 5.00 | | 5.00 | 5.00 | | 2.00 | 5.00 | 5.00 |
| Xanthan gum | | 300 | | | | | 0.50 | 0.30 | 0.30 | | 0.005 |
| Welan gum | | | | | 0.30 | 2.00 | | | | 0.005 | |
| CMC (A) | | | 1.00 | | | | | | 1.00 | | 0.05 |
| CMC (B) | | | | | | | | 500 | | | |
| CMC (E) | | | | | | | 5.00 | | | | |
| Nanolyacrylate (A) | | | | | | | | | | | |
| Na polyacrylate (B) | | | | 1.00 | | | | | | 0.15 | |
| (Calculated amount) | | 67.00 | 59.00 | 74.00 | 19.70 | 53.00 | 54.50 | 54.70 | 87.70 | 22.845 | 54.945 |
| Liquid state | | Unable to be prepared | | | Unable to be prepared | Unable to be prepared | | Unable to be prepared | | | |
| Stationary viscosity | (low shear rate) | | 400 | 2100 | | | 26800 | | 4400 | 87600 | 800 |
| | (high shear rate) | | 340 | 570 | | | 3870 | | 520 | 100000 | 130 |
| After shearing | (low shear rate) | | 350 | 700 | | | 11000 | | 1000 | 100000 | 1200 |
| | (high shear rate) | | 314 | 500 | | | 2300 | | 468 | 6700 | 140 |
| | | | | | | | | | | | |
| At a time of stationary storage | (coefficient a) | | 381 | 1433 | | | 15201 | | 2353 | 91065 | 469 |
| | (coefficient b) | | -0.044 | -0.354 | | | -0.526 | | -0.58 | -0.036 | -0.494 |
| Immediately after the shearing | (coefficient a) | | 339 | 634 | | | 6954 | | 800 | 48892 | 639 |
| | (coefficient b) | | 003 | -0.091 | | | -0.425 | | -0.206 | -0.663 | -0.584 |
| | | | | | | | | | | | |
| Storage stability | | | X | X | | | ⊚ | | ⊚ | ⊚ | X |
| Carburization | | | ⊚ | ⊚ | | | X | | ⊚ | ⊚ | ⊚ |
| Sprayability | (25°C) | | ⊚ | ○ | | | ○ | | ⊚ | X | ⊚ |
| Adhesive property | (80°C) | | X | X | | | ○ | | X | X | X |
| | (80°C) | | X | X | | | ○ | | X | X | X |
| | (100°C) | | X | X | | | ○ | | X | X | X |
| | (120°C) | | XX | XX | | | ○ | | X | X | XX |

| | | | | | | | | | | | |
|---|---|---|---|---|---|---|---|---|---|---|---|
| CMC*(A): molecular weight (100,000), viscosity (800/2%**) CMC*(B): molecular weight (250,000), viscosity (1600/1%**) CMC*(C): molecular weight (175,000), viscosity (2500/2%) CMC*(D): molecular weight (195,000), viscosity (3500/2%) CMC*(E): molecular weight (30,000), viscosity (15/2%) Na polyacrylate (A): molecular weight (500,000), viscosity (75/1%) Na polyacrylate (B): molecular weight (1,650,000), viscosity (300/0.2%) * CMC = Na salt of carboxymethylcellulose **: It means that the viscosity of a 2% solution thereof in water at 25°C was 8000 mPa·s. | | | | | | | | | | | |

### (4) Conclusion

From the above-mentioned test results, it was proved that a lubricant composition of the invention has performances good in all of storage stability, sprayability, and adhesion property. Or the other hand, about the group of a lubricant compositions of Comparative Examples, satisfactory performances therefor were unable to be obtained.

The above has described the invention in connection with embodiments which appear to be most practical and preferable at the present time. However, the invention is not limited to the embodiments disclosed in the specification of the present application, and can be appropriately varied within a scope not contrary to the subject matter and the conception of the invention read out from the claims and the whole of the specification. It should be understood that any lubricant composition for seamless steel pipes or tubes working with such a variation is also included in the technical scope of the invention.

### Industrial Applicability

A lubricant composition for seamless steel pipes or tubes working of the invention is useful for working in the Mannesmann process for producing a seamless steel pipe.

### Brief Description of the Drawings

FIG. 1 is a chart showing an ideal viscosity form as a lubricant composition for seamless steel pipes or tubes working.
FIG. 2 is a view of a chemical structure model of an example of the pseudo plastic fluidity water-soluble polymer.
FIG. 3 is a view showing a chemical structure model of a long-chain polymer wherein glucoses are subjected to glucoside bonding, the polymer being an example of the thixotropic fluidity water-soluble polymer.
FIG. 4 is a chart showing viscosity properties of static and dynamic states of a pseudo plastic fluidity water-soluble polymer.
FIG. 5 is a chart showing viscosity properties of static and dynamic states of a thixotropic fluidity water-soluble polymer.

## Claims

1. A lubricant composition for seamless steel pipes or tubes working, which has a viscosity property represented by the following approximate expression: Y = a·X^{b}
wherein Y: viscosity (mPa·s), X: shear rate (s⁻¹); and
a: 4000 to 40000 and b: -1.0 to -0.3 on measurement of viscosity at 25°C using a Model B viscometer after the lubricant composition has been kept stationary for twenty four hours, and
a: 1000 to 20000, and b: -1.0 to -0.15 on measurement of viscosity at 25°C using a Model B viscometer, 90 seconds after completion of shearing by stirring of the lubricant composition;
wherein measurement after the lubricant composition has been kept stationary comprises the following steps:
• the lubricant composition is stirred and then kept still for 24 hours;
• after 24 hours has passed, viscosity is measured at low shear rate (1.5rpm; shear rate 0.323 to 0.366s⁻¹) using a Model B viscometer.
• 60 seconds after measurement is begun, data is read out from the Model B viscometer and multiplied by a multiplying constant;
• subsequently viscosity is measured at high shear rate (60rpm; shear rate 12.9 to 14.6s⁻¹) using the Model B viscometer;
• 60 seconds after the high shear rate measurement is begun data is read out from the Model B viscometer and multiplied by a multiplying constant;
and wherein measurement of viscosity 90 seconds after completing shearing by stirring comprises the following steps:
• a 500mL sample of the lubricant composition is stirred at 3000 rpm for one minute by means of a propeller of 50mm diameter, shearing by stirring being completed at the time at which rotation of the propeller is stopped;
• 30 seconds from completion of shearing by stirring the viscosity is measured at low shear rate (1.5rpm; shear rate 0.323 to 0.366s⁻¹) using a Model B viscometer.
• 60 seconds after measurement is begun, data is read out from the Model B viscometer and multiplied by a multiplying constant;
• the sample is again sheared by stirring at 3000rpm for one minute by means of a propeller of 50mm diameter, shearing by stirring being completed at the time at which rotation of the propeller is stopped;
• 30 seconds after completion of shearing by stirring viscosity is measured at high shear rate (60rpm; shear rate 12.9 to 14.6s⁻¹) using the Model B viscometer;
• 60 seconds after the high shear rate measurement is begun data is read out from the Model B viscometer and multiplied by a multiplying constant;
wherein measurement 90 seconds after completion of shearing by stirring means beginning the viscosity measurement 30 seconds after completion of shearing by stirring and reading viscosity data 60 seconds after the start of the measurement; and
wherein the lubricant composition comprises 10 to 40% by mass of an oxide-based layered compound, 5 to 30% by mass of one or more alkali metal salts or amine salts of boric acid, 0.11 to 3.0% by mass of one or more water-soluble polymers which are soluble in an aqueous solution of the alkali metal salt(s) or amine salt(s) of boric acid, and water as the balance; the average particle diameter of the oxide-based layered compound being from 1 to 40 mm.

2. The lubricant composition for seamless steel pipes or tubes working according to claim 1, which comprises, as the water-soluble polymer(s), a pseudoplastic water-soluble polymer, or a mixture of a pseudoplastic water-soluble polymer and a thixotropic water-soluble polymer.

3. The lubricant composition for seamless steel pipes or tubes working according to claim 1, which comprises, as the water-soluble polymer(s), a pseudo plastic fluidity water-soluble polymer in an amount of 0.01 to 1.0% by mass of the whole of the lubricant composition, and a thixotropic fluidity water-soluble polymer in an amount of 0.1 to 2,0% by mass of the whole of the lubricant composition.

## Patentansprüche

1. Schmiermittelzusammensetzung für nahtlose Stahlrohre oder Arbeitsrohre, die eine durch die folgende angenäherte Beziehung dargestellte Viskositätseigenschaft hat: $Y = a ⋅ {X}^{b}$
wobei Y: Viskosität (mPa·s), X: Scherrate (s⁻¹); und
a: 4000 bis 40000 und b: -1,0 bis -0,3, beim Messen der Viskosität bei 25 °C unter Verwendung eines Modell-B-Viskosimeters, nachdem die
Schmiermittelzusammensetzung für 24 Stunden stationär gehalten wurde, und
a: 1000 bis 20000 und b: -1,0 bis -0,15, beim Messen der Viskosität bei 25 °C unter Verwendung eines Modell B Viskosimeters, 90 Sekunden nach Abschluss des Scherens durch Rühren der Schmiermittelzusammensetzung;
wobei die Messung, nachdem die Schmiermittelzusammensetzung stationär gehalten wurde, die folgenden Schritte umfasst:
• die Schmiermittelzusammensetzung wird gerührt und dann für 24 Stunden stehen gelassen;
• nach Verstreichen von 24 Stunden wird die Viskosität mit niedriger Scherrate (1,5 U/min; Scherrate 0,323 bis 0,366 s-¹) unter Verwendung eines Modell-B-Viskosimeters gemessen.
• 60 Sekunden nach Beginn der Messung werden die Messwerte aus dem Modell-B-Viskosimeter ausgelesen und mit einer Multiplikationskonstante multipliziert;
• anschließend wird die Viskosität bei hoher Scherrate (60 U/min; Scherrate 12,9 bis 14,6 s⁻¹) unter Verwendung des Modell-B-Viskosimeters gemessen;
• 60 Sekunden nachdem die Messung bei hoher Scherrate begonnen wurde, werden die Messwerte aus dem Model-B-Viskosimeter ausgelesen und mit einer Multiplikationskonstante multipliziert;
und wobei die Messung der Viskosität 90 Sekunden nach Abschluss des Scherens durch Rühren die folgenden Schritte umfasst:
• eine 500- ml-Probe der Schmiermittelzusammensetzung wird bei 3000 U/min für eine Minute mittels eine Propellers von 50 mm Durchmesser gerührt, wobei das Scheren durch Rühren zu einer Zeit abgeschlossen wird, bei der die Drehung des Propellers angehalten wird;
• 30 Sekunden nach Abschluss des Scherens durch Rührens wird die Viskosität bei niedriger Scherrate (1,5 U/min; Scherrate 0,323 bis 0,366 s⁻¹) unter Verwendung eines Modell-B-Viskosimeters gemessen.
• 60 Sekunden nach Beginn der Messung werden die Daten aus dem Modell-B-Viskosimeter ausgelesen und mit einer Multiplikationskonstante multipliziert;
• Die Probe wird erneut durch Rühren bei 3000 U/min für eine Minute mittels eines Propellers von 50 mm Durchmesser geschert, wobei das Scheren durch Rühren zu der Zeit abgeschlossen wird, bei der die Drehung des Propellers angehalten wird;
• 30 Sekunden nach Abschluss des Scherens durch Rühren wird die Viskosität bei hoher Scherrate (60 U/min; Scherrate 12,9 bis 14,6 s⁻¹) unter Verwendung des Modell-B-Viskosimeters gemessen;
• 60 Sekunden nach Beginn der Messung bei hoher Scherrate werden die Daten aus dem Modell-B-Viskosimeter ausgelesen und mit einer Multiplikationskonstante multipliziert;
wobei die Messung 90 Sekunden nach Abschluss des Scherens durch Rühren bedeutet, dass die Viskositätsmessung 30 Sekunden nach Abschluss des Scherens durch Rühren und das Auslesen der Viskositätsdaten 60 Sekunden nach Beginn der Messung begonnen werden;
und
wobei die Schmiermittelzusammensetzung 10 bis 40 Masse-% einer oxidbasierten Schichtverbindung, 5 bis 30 Masse-% von einem oder mehren Alkalimetallsalzen oder Aminsalzen von Borsäure, 0,11 bis 3,0 Masse-% von einem oder mehreren wasserlöslichen Polymeren, die in einer wässrigen Lösung des Alkalimetallsalzes (der Alkalimetallsalze) löslich sind, oder Aminsalz(e) von Borsäure und Wasser als Rest umfasst, wobei der durchschnittliche Teilchendurchmesser der oxidbasierten geschichteten Verbindung 1 bis 40 µm beträgt.

2. Schmiermittelzusammensetzung für nahtlose Stahlrohre oder Arbeitsrohre nach Anspruch 1, die, als das (die) wasserlösliche(n) Polymer(e) ein pseudoplastisches wasserlösliches Polymer oder ein Gemisch von einem pseudoplastischen wasserlöslichen Polymer und einem thixotropen wasserlöslichen Polymer umfasst.

3. Schmiermittelzusammensetzung für nahtlose Stahlrohre oder Arbeitsrohre nach Anspruch 1, das als das (die) wasserlösliche(n) Polymer(e) ein pseudoplastisches wasserlösliches Fluiditätspolymer in einer Menge von 0,01 bis 1,0 Masse-% der Gesamtheit der Schmiermittelzusammensetzung und ein thixotropes wasserlösliches Fluiditätspolymer in einer Menge von 0,1 bis 2,0 Masse-% der Gesamtheit der Schmiermittelzusammensetzung umfasst.

## Revendications

1. Composition de lubrifiant pour l'usinage de tubes ou de tuyaux en acier sans soudure, laquelle présente une propriété de viscosité représentée par l'expression approchée suivante : Y = a.X^{b}
où Y : viscosité (mPa.s), X : vitesse de cisaillement (s⁻¹) ; et
a : 4 000 à 40 000 et b : -1,0 à -0,3 sur la mesure de la viscosité à 25°C en utilisant un viscosimètre modèle B après que la composition de lubrifiant a été maintenue stationnaire pendant vingt-quatre heures, et
a : 1 000 à 20 000, et b : -1,0 à -0,15 sur la mesure de la viscosité à 25°C en utilisant un viscosimètre modèle B, 90 secondes après l'achèvement du cisaillement par agitation de la composition de lubrifiant ;
dans laquelle la mesure après que la composition de lubrifiant a été maintenue stationnaire comprend les étapes suivantes :
• la composition de lubrifiant est agitée et ensuite maintenue au repos pendant 24 heures ;
• après que 24 heures se sont écoulées, la viscosité est mesurée à une faible vitesse de cisaillement (1,5 tr/min ; vitesse de cisaillement de 0,323 à 0,366 s⁻¹) en utilisant un viscosimètre modèle B.
• 60 secondes après que la mesure est commencée, la donnée est lue à partir du viscosimètre modèle B et multipliée par une constante de multiplication ;
• la viscosité est ensuite mesurée à une vitesse de cisaillement élevée (60 tr/min ; vitesse de cisaillement de 12,9 à 14,6 s⁻¹) en utilisant le viscosimètre modèle B ;
• 60 secondes après que la mesure de la vitesse de cisaillement élevée est commencée, la donnée est lue à partir du viscosimètre modèle B et multipliée par une constante de multiplication ;
et dans laquelle la mesure de la viscosité 90 secondes après l'achèvement du cisaillement par agitation comprend les étapes suivantes :
• un échantillon de 500 mL de la composition de lubrifiant est agité à 3 000 tr/min pendant une minute au moyen d'une pale d'agitation de diamètre 50 mm, le cisaillement par agitation étant achevé au moment auquel la rotation de la pale d'agitation est arrêtée ;
• 30 secondes après l'achèvement du cisaillement par agitation la viscosité est mesurée à une faible vitesse de cisaillement (1,5 tr/min ; vitesse de cisaillement de 0,323 à 0,366 s⁻¹) en utilisant un viscosimètre modèle B.
• 60 secondes après que la mesure est commencée, la donnée est lue à partir du viscosimètre modèle B et multipliée par une constante de multiplication ;
• l'échantillon est à nouveau cisaillé par agitation à 3 000 tr/min pendant une minute au moyen d'une pale d'agitation de diamètre 50 mm, le cisaillement par agitation étant achevé au moment auquel la rotation de la pale d'agitation est arrêtée ;
• 30 secondes après l'achèvement du cisaillement par agitation la viscosité est mesurée à une vitesse de cisaillement élevée (60 tr/min ; vitesse de cisaillement de 12,9 à 14,6 s⁻¹) en utilisant le viscosimètre modèle B ;
• 60 secondes après que la mesure de la vitesse de cisaillement élevée est commencée, la donnée est lue à partir du viscosimètre modèle B et multipliée par une constante de multiplication ;
dans laquelle la mesure 90 secondes après l'achèvement du cisaillement par agitation indique le début de la mesure de la viscosité 30 secondes après l'achèvement du cisaillement par agitation et la lecture de la donnée de la viscosité 60 secondes après le début de la mesure ; et
dans laquelle la composition de lubrifiant comprend de 10 à 40 % en masse d'un composé à couches à base d'oxyde, de 5 à 30 % en masse d'un ou plusieurs sels de métaux alcalins ou de sels d'amines d'acide borique, de 0,11 à 3,0 % en masse d'un ou plusieurs polymères solubles dans l'eau qui sont solubles dans une solution aqueuse du(des) sel(s) de métaux alcalins ou du(des) sel(s) d'amine(s) d'acide borique, et de l'eau pour le reste, le diamètre moyen de particule du composé à couches à base d'oxyde étant de 1 à 40 µm.

2. Composition de lubrifiant pour l'usinage de tubes ou de tuyaux en acier sans soudure selon la revendication 1, laquelle comprend, comme le(les) polymère(s) soluble(s) dans l'eau, un polymère soluble dans l'eau pseudoplastique, ou un mélange d'un polymère soluble dans l'eau pseudoplastique et d'un polymère soluble dans l'eau thixotrope.

3. Composition de lubrifiant pour l'usinage de tubes ou de tuyaux en acier sans soudure selon la revendication 1, laquelle comprend, comme le(les) polymère(s) soluble(s) dans l'eau, un polymère soluble dans l'eau de fluidité pseudoplastique dans une quantité de 0,01 à 1,0 % en masse de la totalité de la composition de lubrifiant, et un polymère soluble dans l'eau de fluidité thixotrope dans une quantité de 0,1 à 2,0 % en masse de la totalité de la composition de lubrifiant.
